

# UNITED STATES PATENT OFFICE.

JAMES P. ELLIOTT, OF OAK PARK, ILLINOIS; MARY BRODERS ELLIOTT EXECUTRIX OF  
SAID JAMES P. ELLIOTT, DECEASED.

## PROCESS OF MAKING INSULATING AND BRINE AND WATER PROOF MATERIAL.

1,406,174.

Specification of Letters Patent. Patented Feb. 14, 1922.

No Drawing.

Application filed November 23, 1917. Serial No. 203,508.

To all whom it may concern:

Be it known that I, JAMES P. ELLIOTT, a citizen of the United States, residing at Oak Park, county of Cook, State of Illinois, have 5 invented a certain new and useful Improvement in Processes of Making Insulating and Brine and Water Proof Material, and declare the following to be a full, clear, and exact description of the same, such as will 10 enable others skilled in the art to which it pertains to make and use the same.

In my prior Patent No. 1,305,081, granted May 27, 1919, I have disclosed a new process of making a body or sheet of fibrous 15 material saturated and coated with asphaltum. For some purposes it is desirable that the coating have characteristics different from those possessed by ordinary saturating compounds. Thus for example, where it is 20 desirable to give the sheet or body a high finish it is necessary to have a coating material which will be hard enough for this purpose and insoluble enough to resist the solvents that may be contained in varnishes, 25 paints or enamels that may be applied thereto.

The object of my present invention is to produce a fibrous sheet or body of the kind referred to in my aforesaid patent but having 30 a hard coating capable of offering a high degree of resistance to the action of solvents and of taking a high finish.

In carrying out my invention I intimately mix with wet pulp any desired percentage of 35 finely divided hard asphaltum, usually a very large proportion of dry asphaltum to dry pulp, and then press the pulp into shape. The pressure not only gives the desired shape to the sheet or body but it also makes it 40 dense and expels the water therefrom. After the product leaves the press I coat it with baking or stoving japan and bake it in an oven whose temperature is higher than the melting point of the asphaltum contained 45 in the product. This operation melts the asphaltum and changes it from a powdery state to a single coherent mass throughout which the fibrous material is distributed. During the first stages of the baking the 50 moisture is expelled and, because it takes a long time for the japan to become dry or set, the moisture passes out through the japan and while the latter is still in a liquid state. Consequently the moisture escapes readily and prior to the time that the

japan assumes a state which will prevent it from flowing and closing the openings made by the escaping bubbles of air and moisture, and, when the japan dries and sets, it forms a continuous impervious coating. 60

The fiber in the mass ties the asphaltum together even at high temperatures. Therefore, my improved product is stronger, tougher and more durable than one made of asphaltum alone would be, and, at the same 65 time, it has a surface coating which it would be impossible to place on a body made of asphaltum alone because such a body could not retain its shape during the baking process but would melt and flow. It will also be 70 seen that the fibers are all thoroughly coated by the asphaltum in addition to being enveloped in the japan coating, and therefore my improved product will be as thoroughly 75 resistant to all agencies which asphaltum will resist as though the interior thereof were made of asphaltum alone.

While for many purposes asphaltum will be the most desirable material for mixture with the pulp, other materials such as rosin, 80 natural and artificial waxes or gums, may be employed to advantage as substitutes for the asphaltum.

I claim:

1. The process which consists in intimately mixing wet pulp with finely-divided asphaltum, compressing the wet mixture under heavy pressure without a preliminary application of heat, then coating the mass with baking or stoving japan, and finally 90 baking the mass at a temperature high enough to melt the asphaltum. 85

2. The process which consists in intimately mixing with wet pulp finely-divided fusible material capable of resisting the action of acids and brines and having insulating properties, then pressing the wet mixture under heavy pressure, then coating the mass with baking or stoving japan, and finally baking the mass at a temperature 100 high enough to fuse said material. 95

3. The process which consists in intimately mixing with wet pulp finely-divided asphaltum, compressing the wet mixture so as to compact the same and drive out a large 105 part of the water without changing the character of the asphaltum, coating the compressed mass with baking or stoving japan, and finally baking the mass at a temperature high enough to melt the asphaltum so as si- 110

multaneously to melt the asphaltum, drive out the moisture and bake the japan.

4. The process which consists in intimately mixing with wet pulp finely-divided fusible material capable of resisting the action of acids and brines and having insulating properties, compressing the wet mixture so as to drive out a large part of the water

without changing the character of said fusible material, coating the mass with baking or 10 stoving japan, and baking the mass at a temperature high enough to fuse said fusible material.

In testimony whereof I sign this specification.

JAMES P. ELLIOTT.